

Patented Oct. 11, 1927.

1,644,764

# UNITED STATES PATENT OFFICE.

LEO WALLERSTEIN, OF NEW YORK, N. Y., ASSIGNOR TO WALLERSTEIN COMPANY, INC.,  
OF NEW YORK, N. Y., A CORPORATION OF NEW YORK.

## PROCESS OF DEGUMMING SILK.

No Drawing. Application filed April 15, 1922, Serial No. 553,279. Renewed February 24, 1926.

This invention relates to a process for degumming silk.

The object of the invention is to provide a process which will be more economical than the processes heretofore known and which may be carried out in practice with ordinary care without danger of injury to the silk.

With this general object in view, the invention broadly considered comprises a treatment of the silk with a solution of a proteolytic enzyme which is active in an acid, in a slightly alkaline, and in a neutral medium. While there are a number of such proteolytic enzymes which may be used, the proteolytic enzyme known in commerce as papain is especially suitable for the purposes of this invention.

I now give some specific example of the manner of carrying out my invention.

The raw silk may be subjected first to the action of a weak soap solution, as, for example, a solution containing  $\frac{1}{4}\%$  soap. While the amount of such solution relative to the amount of raw silk may vary and need only be such as to permit the convenient washing and working of the silk, it is advisable to so proportion the bath that the total soap therein will be about 2 to 5 per cent of the weight of the raw silk to be treated. This bath is kept at a temperature of 70 to 95° C., and the raw silk is allowed to remain in the bath for about 5 to 15 minutes. This bath is a rinsing bath for the purpose of removing any surface dirt, oils, and impurities. At the end of this treatment the silk is removed and the water pressed out in any suitable manner, as, for example, by a wringer or a centrifuge.

Instead of this soap solution some other weakly alkaline solution may be employed, as, for example, a weak solution of sodium carbonate or bicarbonate.

The silk is then immersed in a very weak solution of papain. This solution is made in the proportion of 1 gm. of papain to 4 to 5 liters of water. When the silk is first immersed, the bath should be at a temperature of about 50 to 70° C., but the temperature is best raised to about 75° C. after the silk has been in the bath for a few minutes. The bath is stirred at frequent intervals and the silk is worked over in the usual way so as to make sure that the solution

comes into intimate contact with all parts of the silk. The silk is kept in this for about one to two hours, at the end of which time it is removed to a rinsing bath of clean water, thoroughly rinsed and then dried. Instead of rinsing in clean water, the silk may be rinsed in a weak soap solution and then dried. By the use of this treatment, viz, rinsing in a soap solution, the lustre and "feel" of the silk are enhanced. If the silk is to be dyed at once, it may be rinsed in the clean water or soap bath after removal from the papain solution, as described above, and then may go directly to the dyeing bath, which may contain some soap.

I have given the proportions of the papain solution as 1 gm. of papain to 4 to 5 liters of water and the time of treatment as about one to two hours, but this is based on the assumption that the papain is of the normal commercial strength or activity. It is to be understood that variations in the proportions and in the time of treatment may be necessary where the papain varies from the normal standard. The proportion of papain used depends on its activity and on its time of action, as well as on the condition of the silk.

In another example of the process, the degumming bath itself may contain soap. For example, papain may be added to a  $\frac{1}{4}\%$  per cent soap solution in the proportion of 1 gm. to 4 to 5 liters of soap solution. In this bath the silk is immersed and allowed to stay for 1 to 3 hours, the bath being kept at a temperature of about 50° C. when the silk is first immersed therein and may then be gradually raised to 75° C.

The silk may be worked over in the usual way, and when sufficiently degummed may be moved to a rinsing bath of clean water, rinsed, removed and dried. Or it may be given a treatment in another weak soap bath.

Also, it may be advantageous to add to the water solution of papain a weak organic acid, for example, acetic acid, so that the resulting bath is slightly acid to litmus. The treatment of the silk in this bath is followed by a treatment in a weak soap solution. The use of the slightly acid papain bath tends to make the fibre tougher.

Instead of limiting the temperature of the papain and soap bath to 50 to 75° C., as stated above, it is sometimes advanta-

geous to quickly raise the bath to 95° C. for a short time prior to removal of the silk to the rinsing bath.

By using a proteolytic enzyme which is active in all three classes of media, viz, acid, neutral and slightly alkaline, there is no danger of the enzyme action being stopped by changes in the degree of acidity or alkalinity of the bath, such as might occur in practice, and also it becomes possible to use soap or acids with the enzyme in the bath, as hereinbefore pointed out.

What is claimed is:

1. The process of degumming silk, which comprises subjecting the silk to the action of a proteolytic enzyme of that type which is active in a neutral, as well as a weakly alkaline and a slightly acid medium, at a temperature not less than 50° C.

2. The process of degumming silk, which comprises immersing it in a bath containing water and a proteolytic enzyme of that type which is active in a neutral as well as a weakly alkaline and a slightly acid solution, and gradually increasing the temperature of the bath from about 50° C. to about 75° C.

3. The process of degumming silk, which comprises immersing it in a bath containing water and a proteolytic enzyme of that type which is active in a neutral as well as a weakly alkaline and a slightly acid solution, gradually increasing the temperature of the bath from about 50° C. to about 75° C., and then quickly raising the temperature to 95° C. for a short time before removing the silk from the bath.

4. The process of degumming silk which comprises immersing the silk in a bath containing water and a proteolytic enzyme of that type which is active in a neutral, in a weakly alkaline and in a slightly acid solution, said bath being maintained at a temperature not less than 50° C., allowing the silk to remain in the bath until sufficiently

degummed, and then removing the silk, rinsing and drying it.

5. The process of degumming silk which comprises subjecting it to the action of a solution of papain at a temperature sufficient to maintain the activity of the enzyme, until the desired amount of degumming has occurred.

6. The process of degumming silk which comprises subjecting it to an aqueous solution containing papain in the proportion of about 1 gm. of papain to 4 to 5 liters of water, the bath being at about 50° to 70° C. when the silk is entered, gradually raising the temperature of the bath to about 75° C., and keeping the silk therein for about 1 hour.

7. The process of degumming silk which comprises first washing the silk in a soap solution then rinsing the silk, immersing it in a bath comprising an aqueous solution of a proteolytic enzyme of that type which is active in a neutral, in a weakly alkaline and in a slightly acid medium, maintaining the bath at a temperature of 50° to 75° C. until the silk is sufficiently degummed, and then removing the silk from the bath.

8. The process of degumming silk which comprises subjecting it to the action of a weak soap solution containing papain, while maintaining the solution at a temperature sufficient to maintain the activity of the enzyme, until the desired amount of degumming has occurred.

9. The process of degumming silk which comprises subjecting it to the action of a solution containing papain and about  $\frac{1}{4}$  to  $\frac{1}{2}\%$  soap, while maintaining the solution at a temperature sufficient to maintain the activity of the enzyme, until the desired amount of degumming has occurred.

In testimony whereof, I have hereunto set my hand.

LEO WALLERSTEIN.